

## UNITED STATES PATENT OFFICE.

CARL D. PRATT, OF TAMAQUA, PENNSYLVANIA, ASSIGNOR TO ATLAS POWDER COMPANY, OF WILMINGTON, DELAWARE, A CORPORATION OF DELAWARE.

## BLASTING-POWDER COMPOSITION.

No Drawing.

Application filed May 31, 1924. Serial No. 717,140.

*To all whom it may concern:*

Be it known that CARL D. PRATT, citizen of the United States, residing at Tamaqua, in the county of Schuylkill and State of Pennsylvania, has invented certain new and useful Improvements in Blasting-Powder Compositions, of which the following is a specification.

My invention relates to improvements in blasting powder compositions, and it has for its object to provide a new and highly useful commercial blasting explosive which will possess characteristics of safety far beyond those of ordinary black blasting powder.

The record of the Bureau of Mines of the United States, covering the period from 1908 to 1923 shows that seventy-one coal mine explosions have been caused directly by the use of black blasting powder or by black blasting powder and dynamite, killing more than eight hundred men, injuring many others and causing untold property damage. This serious situation can be largely corrected by the substitution, for black blasting powder, of what are known as "permissible" explosives, that is explosives which have passed certain tests prescribed by the Bureau of Mines. Tests conducted by said bureau, and verified in actual coal mining operations, have demonstrated conclusively that a permissible explosive has a very much shorter and cooler flame than black blasting powder and a very much cooler flame than any other high explosive.

With the foregoing facts in mind it has been my aim to provide a series of blasting powder compositions, which have decreased tendencies, compared with current commercial grades of blasting powder, to ignite inflammable gases and dusts or mixtures thereof; as for example, those occurring in coal mines.

It should be expressly understood that my invention is not concerned with so-called "high explosives", but is concerned entirely with the type of so-called "low explosives", herein referred to as "blasting powders".

"High explosives" include both individual compounds and mixtures of ingredients, which are able to suddenly decompose in the manner of a detonation, through almost instantaneous disintegrations and re-

actions, as influenced by heat or shock or both. "Low explosives", on the other hand, consist only of mixtures of ingredients, of such nature as to react with each other, in the form of a rapid combustion, as distinguished from a sudden disintegration, when influenced by heat. It is a peculiarity of "high explosives" that they decompose with a much higher speed than "low explosives", thus exerting quicker and more disruptive actions than the slower and consequently more propulsive "low explosives".

My improved blasting powders may, properly, be referred to as "safety blasting powders," since they are safer for use under gaseous and dusty conditions, such as coal-mining, than the current blasting powders, just as permissible high explosives are safer for use in coal-mines than straight nitroglycerine dynamites or gelatins.

As a result of a very exhaustive study of many principles and extensive experimentation in following out these principles in a very large number of mixtures, I have been able to devise a series of blasting powders, with decreased tendencies, (compared with current commercial blasting powders) to ignite inflammable gases and dusts (or mixtures thereof); through the discovery that carbohydrates and metallic and ammonium chlorides, when added to blasting powder compositions, consisting of one or more metallic nitrates, sulphur and one or more materials that are essentially carbon, will effectively produce these improvements in combination or singly.

Carbohydrates, I have found, such as sugar, cellulose, glucose, starch and the like, produce the desired decreased tendencies to ignite inflammable gases and dusts or mixtures thereof, through their introduction into the chemical constitutions of blasting powders, of greater amounts of carbon and hydrogen in proportion with oxygen, to the extent of markedly decreasing the amounts of heat evolved by the decomposition reactions of such compositions.

I have also found that metallic and ammonium chlorides, such as sodium chloride, potassium chloride, barium chloride, ammonium chloride and the like, produce the desired decreased tendencies to ignite inflammable gases and dusts or mixtures there-

of, when in intimate contact with the decomposition reactions of blasting powder compositions,—especially those including one or more carbohydrates,—through their 5 heat absorbing abilities.

Further, I have discovered that blasting powder compositions, including carbohydrates and metallic and ammonium chlorides, in combination, or singly, to suit requirements, together with the usual blasting powder ingredients, (metallic nitrates, sulphur and materials that are essentially carbon), will actually have several times less 10 tendency to ignite inflammable gases and 15 dusts or mixtures thereof, than the current commercial grades of blasting powders. That is, charges of my "safety blasting powders" (hereinbefore defined) that I am able to fire into certain inflammable gases 20 and dusts or mixtures thereof, without igniting them, are several times the weight of current commercial blasting powder charges, which will ignite the same inflammable gases and dusts or mixtures thereof, under like 25 conditions.

It should be expressly understood that the scope of my invention is broad enough to include any manner of introduction of the cooling ingredients; namely carbohydrates 30 and metallic and ammonium chlorides. That is, the said cooling ingredient or ingredients may be introduced in various manners, to suit conditions; as for instance, actual incorporation with the other ingredients or incorporation with only a portion of the other 35 ingredients or included as separate granules but mixed with granules of the other ingredients or with the grains of commercial grades of blasting powders, etc.

It should also be expressly understood that the scope of my invention is not limited to any particular physical form of "safety blasting powders." That is, the physical form of said "safety blasting powders" may 40 vary in any manner whatsoever, to suit commercial application; as for instance, granules, pellets, powders, cubes, cylinders, etc.

Summarizing, my "safety blasting powders" consist of one or more carbohydrates 50 in any practicable quantity (preferably from 5 to 35%) and one or more metallic or ammonium chlorides (preferably from 1 to 15%), used in combination or singly with practicable combinations of metallic nitrates, sulphur and materials that are essentially 55 carbon. Other ingredients may also be added to the above in minor quantities and still be within the scope of my invention; such as organic or inorganic compounds, that will absorb heat through the reduction of oxygen or by their volatilization 60 during the decomposition reactions or by their liberation of water of crystallization or combination of such causes.

Typical formulæ, by way of examples, are: 65

|                   | Per cent. |    |    |    |
|-------------------|-----------|----|----|----|
| Sodium nitrate    | 54        | 44 | 54 | 47 |
| Potassium nitrate |           | 10 |    | 8  |
| Sugar             |           | 10 |    | 20 |
| Starch            | 23        | 13 | 17 | 70 |
| Sulphur           |           | 4  | 4  | 5  |
| Charcoal          | 19        | 15 | 17 | 14 |
| Lignite           |           |    | 4  |    |
| Sodium chloride   |           |    | 7  | 4  |
|                   |           |    |    | 75 |

My investigations indicate that I may vary the physical characteristics of my improved "safety blasting powders" through variation of their densities, granulations, physical forms, etc., and produce similar effectiveness to the grades of blasting powders now used in the coal-mines of the United States with the advantage of being less apt to cause the very terrible coal-mine disasters that occur when inflammable gas and dust mixtures, contained therein, are ignited. I may also see fit to add other ingredients to my "safety blasting powders," as hereinbefore defined, in order to produce the most desirable combinations of effectiveness and safety.

If carried into effect, through substitution of the above described "safety blasting powders" for all the present types of so-called blasting powders, used in American coal mines, my invention will cause the improvement, hereinbefore described, of over 70% of all the explosives, used for blasting coal in the United States.

(See United States Bureau of Mines Technical Paper #340—page 9.)

Having described my invention, what I claim is:

1. An explosive of the character described 105 consisting of the constituents of black blasting powder, from 5 to 35% of carbohydrates, and from 1 to 15% of a metallic chloride.

2. A blasting powder of the class described 110 consisting of a metallic nitrate, sulphur and carbon, the whole constituting black blasting powder to which combination is added from 5 to 35% of carbohydrates and 1 to 15% of a metallic chloride.

3. A blasting powder of the class described 115 consisting of a metallic nitrate, sulphur and a material that is essentially carbon to which combination is added a carbohydrate and a metallic chloride.

4. A blasting powder of the character described 120 consisting of a metallic nitrate, sulphur and a material that is essentially carbon, the whole constituting a black blasting powder to which combination is added from 5 to 35% starch and sugar and 1 to 15% sodium chloride.

In testimony whereof he affixes his signature.

CARL D. PRATT.